

C. S. MORSE.

METHOD AND MEANS FOR BILLET CASTING.

APPLICATION FILED JUNE 8, 1920.

1,387,291.

Patented Aug. 9, 1921.



# UNITED STATES PATENT OFFICE.

CHARLES S. MORSE, OF ROLAND PARK, MARYLAND, ASSIGNOR TO BALTIMORE TUBE COMPANY, INCORPORATED, A CORPORATION OF VIRGINIA.

## METHOD AND MEANS FOR BILLET-CASTING.

1,387,291.

Specification of Letters Patent.

Patented Aug. 9, 1921.

Application filed June 8, 1920. Serial No. 387,348.

To all whom it may concern:

Be it known that I, CHARLES S. MORSE, a citizen of the United States, residing at Roland Park, in the county of Baltimore, State 5 of Maryland, have invented a new and useful Method and Means for Billet-Casting, of which the following is a specification.

My invention relates to hollow billet casting. The object is to provide method and 10 means for casting hollow billets for metal working.

The invention comprises improved method and means for forming or casting a hollow billet, for example in form most desirable 15 for tube making, at minimum expense of labor and material, and with a minimum of defects or imperfections.

The invention is especially adapted for metals and metal alloys of copper, brass and 20 the like, but is applicable also to other metals.

The method now generally employed of casting hollow billets of the alloys above mentioned, is to use a core of yielding material, such as a combination of sand and other substance, so that, as the metal casting cools and contracts, the core will yield sufficiently to permit such contraction, without cracking or other injury to the casting. This practice 25 30 has many disadvantages; for example, this core is difficult and expensive to make and is easily damaged, which results in many defective castings.

In accordance with the present invention 35 the casting is made about a rigid metallic, perfectly formed core, which may be used many times without injury thereto, and is as indestructible as the iron mold itself.

The following method is provided for allowing the contraction of the casting without injury thereto.

The amount of contraction of the molten metal forming the casting, as it cools sufficiently to permit the withdrawal of the core, 40 is calculated, having regard to the mass or volume of metal in the casting and to the composition of the alloy; and the core is so tapered and is withdrawn at a rate of speed corresponding to or compensating for the 45 50 degree of contraction. That is to say, the larger end of the core is the first part withdrawn from the casting, so that the part of the core within the casting becomes smaller and smaller in cross-section as the casting is

poured and contracts, thus permitting the 55 natural contraction of the casting without injury thereto, and the inner surface of the casting is maintained perfectly smooth and without blemish.

It should also be noted that when the 60 molten metal comes into contact with the core, which is comparatively cool, the engaging surface of the casting hardens sufficiently to hold the body of the casting until it solidifies. This permits of a slight lee- 65 way in withdrawing the core.

The following factors therefore enter into a successful practice of my method.

1. The volume of metal forming the casting.

2. The composition of the alloy.

These two factors determine the amount or coefficient of shrinkage or contraction in diameter of the inner wall of the casting.

3. The taper of the core.

4. The speed of withdrawal of the core.

These two factors are co-related with the amount of said contraction. That is to say, the degree of taper of the core and the speed of its withdrawal are dependent, in their 80 calculation, upon said degree or coefficient of contraction of the metal of the casting.

Referring to the drawings, which illustrate merely by way of example, suitable means for effecting my invention:—

Figure 1 is a view in longitudinal section, showing the parts in position at the beginning of the casting operation.

Fig. 2 is a similar view with the core partially withdrawn.

Fig. 3 is a longitudinal section of the mold element with the billet or casting now ready, to be ejected.

Similar numerals refer to similar parts throughout the several views.

The mold element 7 is shown mounted on trunnions 8, adapted to be supported by any suitable means. The tapered core 9 is movably supported therein. The mold element 7 is provided at the top with the removable 100 pouring funnel 10, and at the bottom with the removable block 12, locked in place by the bolt 13.

The core 9 is mounted on or disengagably secured to the rod 14 connected with 105 a piston or plunger 15 operating in the hydraulic cylinder 16. This cylinder is provided with the usual two-way regulating

valve 17 or other suitable means for controlling the speed and direction of movement of the plunger 15 and core 9, as required.

In operation, the metal is poured through

5 funnel 10 into the space 11, between mold

7 and core 9, and the core is withdrawn from the mold by operating the plunger 15, at a speed fixed as above described. The core is made longer than the mold, so that

10 the entire casting is poured and completed before the top of the core drops below the top of the mold. After the core has been withdrawn entirely from the mold 7, and the casting has sufficiently cooled, the funnel

15 10 and block 12 are removed from the mold element 7, and the casting is then ejected therefrom.

The core is preferably permitted to cool before it is again used, in order that the

20 molten metal, when it comes in contact with the core, will harden, as to its contacting or inner surface, sufficiently to hold the body of the casting after the core is withdrawn therefrom, and until the body of the casting

25 solidifies. The core being made of iron or of some metallic compound can be inserted in the mold at a desirable temperature much warmer in fact than can be obtained from a sand core, for the reason that a sand core

30 varies in dampness and temperatures as well as having other undesirable qualities. The iron core can be dressed or coated with a prepared compound the same as the inside surface of the mold, thereby insuring a bet-

35 ter surface on the inside of the hollow billet than can be obtained from a sand core. This is particularly true with some of the copper alloys that are used in seamless tubing in large quantities.

40 While I have described and illustrated, in the foregoing example given, as suitable means for effecting my invention, a stationary mold and movable core, it will be obvious that the core may be stationary and the

45 mold movable for securing the withdrawal of the core from the mold, without departing from the spirit of my invention as defined in the claims.

What I claim is:—

50 1. The method of casting hollow billets which consists in introducing the molten metal into the space formed between a mold element and a separable tapered core element and withdrawing the core element

55 from the mold element while pouring, the degree of taper of the core element and the speed of its withdrawal being dependent upon the degree of contraction of the metal of the casting in the process of cooling.

60 2. The method of casting hollow billets which consists in introducing the molten metal into the space formed between a mold element and a separable tapered core element and withdrawing the core element

65 from the mold while pouring element, the

degree of taper of the core element and the time required in its withdrawal being dependent upon the degree of contraction of the metal of the casting in the process of cooling.

70

3. The method of casting hollow billets which consists in introducing the molten metal into the space formed between a mold element and a separable tapered core element and withdrawing the core element

75

from the mold element while pouring, the degree of taper of the core element and the speed of its withdrawal being dependent upon the degree of contraction of the metal of the casting in the process of 80 partial cooling.

4. The combination of a mold element, a coöperating tapered core element, and means for withdrawing the core element from the mold element while pouring, the degree of 85 taper of the core element and the time of operation of the withdrawing means being dependent upon the degree of contraction of the body of metal cast in the mold, during the process of cooling.

90

5. The combination of a mold element, a coöperating tapered core element, and means for withdrawing the core element from the mold element while pouring, the degree of 95 taper of the core element and the time of operation of the withdrawing means being dependent upon the degree of contraction of the body of metal cast in the mold, during the process of cooling of its inner surface sufficiently to hold the body of the metal.

100

6. The combination of a mold element, a coöperating rigid tapered core element, and means for withdrawing the core element from the mold element while pouring, the degree of taper of the core element and the time of 105 operation of the withdrawing means being dependent upon the degree of contraction of the body of metal cast in the mold, during the process of cooling.

7. The combination of a mold element, a coöperating tapered core element, and means for withdrawing the core element from the mold element while pouring, the degree of 110 taper of the core element and the time of operation of the withdrawing means being 115 dependent upon the coefficient of contraction of the body of metal cast in the mold, during the process of cooling.

8. The combination of a mold element, a coöperating tapered core element, longer 120 than the mold element and adapted, in initial position, to project above the top of the mold element, and means for withdrawing the core element from the mold element, the degree of taper of the core element and 125 the time of operation of the withdrawing means being relative to the degree of contraction of the body of metal cast in the mold, during the process of cooling.

9. The combination of a mold element, a 130

coöperating tapered core element, and means for causing the withdrawal of the core element from the mold element through the lower end of said mold element, said withdrawing means operating in such relation to the pouring of the metal into the mold, that the pouring is completed before the top of

the core passes below the top of the mold, the degree of taper of the core element and the time of operation of the withdrawing means <sup>10</sup> being relative to the degree of contraction of the body of metal cast in the mold, during the process of cooling.

CHARLES S. MORSE.